

**3,524,816**  
**POLYETHER COMPOSITIONS USEFUL AS**  
**HYDRAULIC FLUIDS**

**HYDRAULIC FLUIDS**

**Hugh J. Hagemeyer, Jr., Alden E. Blood, and James D. Heller, Longview, Tex., assignors to Eastman Kodak Company, Rochester, N.Y., a corporation of New Jersey**

**No Drawing. Filed Sept. 6, 1966, Ser. No. 577,185**

**Int. Cl. C09k 3/02**

U.S. Cl. 252—73

U.S. Cl. 252—73

## 4 Claims

## **ABSTRACT OF THE DISCLOSURE**

A mixture of polyethers having the general formulae

$$(1) \quad \text{HOCH}_2\text{CH}_2\text{O}(\text{CH}_2\text{CH}_2\text{O})_x\text{CH}_2\text{CH}_2\text{OH}$$

and



wherein  $x$  is a whole number of from 1-10, said mixture being useful as components of hydraulic fluids.

## DISCLOSURE

This application relates to methods and materials for the production of hydraulic fluids and hydraulic fluid components. More particularly, this invention relates to polyether brake fluid components and brake fluids containing such polyether components.

In commercial brake fluids a very delicate balance of properties is required in order that the finished fluids meet the rigid requirements set up by the Society of Automotive Engineers, hereinafter referred to as SAE. Because of this very delicate balance of properties the substitution of components which are ordinarily considered similar in chemical and physical properties for those used in previously known brake fluids often results in fluids which are unsatisfactory according to SAE standards. Moreover, variation in the amounts of components also frequently results in fluids that are unsatisfactory according to SAE standards.

Acceptable brake fluids are multi-component fluids which contain various ingredients to fulfill the function of a base lubricant, rubber swell inhibitor, viscosity improver, solvent, coupler, and antioxidant. For the most part, brake fluids have conventionally been mixtures of alcohols and glycols in which minor amounts of other addenda are utilized to perform the specific functions such as those of an antioxidant. More recently the use of ethylene oxide adducts of ethylene glycol has been accepted in the trade. Because of the viscosity problems presented by use of the pure adduct, modified reaction products have been frequently utilized. One of the more common modifications is the utilization of some propylene oxide in the adduct. This results in a random mixture which has improved viscosity characteristics. The utilization of such adducts, however, is associated with the normal problems involved with maintaining the delicately restrictive component ratios. Ever increasing demands for improved brake fluids have stimulated continued research efforts directed to meeting such demands.

It is therefore one object of this invention to produce novel polyether brake fluid components. Another object is to produce brake fluid components which allow wider variation in brake fluid component ratios. Another object of this invention will be to provide brake fluids containing novel polyether components. Still another object of this invention is to produce brake fluids in which the

specific fluid components can be varied to a greater degree and yet meet the rigid SAE specifications. Still another object is to provide brake fluid components which perform a dual function, more particularly to perform the function of a hydraulic fluid base lubricant and a rubber swell inhibitor. Still another object is to provide brake fluids having improved volatility characteristics and having excellent viscosity properties.

These and other objects of the invention which will become apparent hereinafter are accomplished by the utilization of an ethylene oxide adduct of ethylene glycol containing a modifying amount of 2,2,4-trimethylpentanediol-1,3. These adducts are generally prepared by reacting the trimethylpentanediol with the ethylene glycol and ethylene oxide, particularly when these materials are present in the reaction mixture in a ratio of from 0.5-2.0 to 3.0-4.5 to 12-24 mole ratio respectively. The reaction is generally catalyzed with an acid or basic catalyst such as Lewis acids, sulfuric acid, benzene sulfonic acid, Raney nickel, sodium hydroxide, boron trifluoride and piperidine. It has been found that trialkyl amines are particularly useful catalysts in that their presence in the resultant product is not detrimental in brake fluids. The reaction is most preferably carried out in an inert environment such as under nitrogen gas and is normally conducted at an elevated temperature of about 75 to 125° C., preferably at 100-115° C. At that temperature range the reaction is normally complete within a two to five hour period but usually is complete in about 3½ hours. The ethylene oxide utilized in the reaction is most advantageously added gradually to the reaction mixture and upon final addition the reaction mixture is allowed to cool slowly and is then filtered.

The filtered product from the reaction scheme outlined above using a trialkylamine catalyst, e.g. triethylamine, has the advantage of being sufficiently pure to obviate any further purification step. The product may be used directly in brake fluids. The product comprises a mixture of compounds having the structural Formulas I and II.

$$\begin{array}{ll}
 \text{(I)} & \text{HOCH}_2\text{CH}_2\text{O}(\text{CH}_2\text{CH}_2\text{O})_x\text{CH}_2\text{CH}_2\text{OH} \\
 \text{(II)} & (\text{CH}_3)_2\text{CH}-\overset{\text{O}}{\underset{\text{H}}{\text{CH}}}-\text{C}(\text{CH}_3)_2\text{CH}_2\text{O}(\text{CH}_2\text{CH}_2\text{O})_x\text{H}
 \end{array}$$

45 wherein  $x$  is a whole number of from 0 to 10, the average value of  $x$  being 3 to 4, and wherein the mixture contains at least some polyethers of Formula I and at least some of Formula II. The relative amounts of the polyethers of Formula I as compared to those of Formula II generally range in the area of from 1-1 to 2-1.

The following specific example is indicative of the general method which can be used in the preparation of the above described adducts.

### EXAMPLE 1

To a 2-liter, 3-necked flask there was added 1 mole of 2,2,4-trimethylpentanediol-1,3; 4 moles of ethylene glycol; and 40 ml. of triethylamine. The reaction vessel was then fitted with condensers, addition funnels, thermowell, and 60 a stirring rod with water-cooled bearing. The reactor was purged with  $N_2$  and the contents heated to 100° C. The addition of 18 moles of liquid ethylene oxide was then started and carried out over a 3½ hour period. The reaction becomes exothermic after the addition of ca. 75 ml. 65 of ethylene oxide, and the reaction temperature is controlled at 100–115° C. After final addition, the reaction product is allowed to cool slowly and is then filtered. No stripping or additional processing is required before utilizing the product as a hydraulic fluid base lubricant- 70 rubber swell inhibitor.

The adduct mixture prepared from Example I is advantageously utilized in the preparation of brake fluids.

The composition has the advantage of performing the dual functions of a base lubricant and a partial rubber swell inhibitor. It has been found that such preparation when mixed with other normal brake fluid components allows for wider variation in the ratios of the individual components. The total brake fluid has properties which fall well within the requirements for the two broad commercial classifications, 70R1 heavy duty and 70R3 extra heavy duty, i.e. classifications which meet the different SAE specifications according to those set forth in SAE procedure J70B-Hydraulic Brake Fluids. With the exception of specialized military hydraulic fluids, all brake fluids fall into these two commercial classifications. The main difference in the specifications for the classifications lies in the requirements for boiling point and flash point.

The brake fluids according to this invention comprise a substantial amount of the trimethylpentanediol/ethylene glycol/ethylene oxide adduct described in combination with various alcohols such as mixed amyl and hexyl alcohols, diethylene glycol monomethyl ether, hexylene glycol, diethylene glycol, mixed heptyl alcohols, 2-methylpentanol, mixed amyl alcohols; and various Cellosolves, such as ethylene glycol monoethyl ether, ethylene glycol monobutyl ether, and ethylene glycol monoisobutyl ether and esters such as 2,2,4-trimethylpentane-1,3-diacetate. The concentration of the trimethylpentanediol adduct in the

(butyl amines and tert butyl hydroquinone) to produce a homogeneous, clear yellow fluid. This fluid was subjected to evaluation as a hydraulic fluid under SAE J70B specifications for 70R1 heavy duty brake fluids. This fluid met all requirements set forth by the specifications. The major results of this evaluation were as follows:

TABLE 1

|    |                                      | Fluid | SAE requirements max. |
|----|--------------------------------------|-------|-----------------------|
| 10 | -40° F. viscosity (centistokes)..... | 1620  | 1800                  |
|    | Flash point, °F.....                 | 157   | 145.5                 |
|    | Percent evaporation (212° F.).....   | 78    | 80                    |
|    | Natural rubber swell (in.).....      | 0.035 | 0.055                 |
|    | SBR rubber swell (in.).....          | 0.030 | 0.055                 |

<sup>1</sup> Min.

These examples that follow represent formulations selected from a wide range of possible compositions of each fluid type. Each example shows variations in some of the fluid components to illustrate the use of the newly developed base lubricant in either 70R1 or 70R3 brake fluids. Each formulation also contains corrosion and oxidation inhibitors, e.g. the secondary amines and di-tertiarybutyl hydroquinone previously mentioned.

The examples below indicate that when components are held within the desired ranges indicated above all SAE specifications are met.

| Component                              | Example No. |       |       |       |       |       |       |       |       |       |      |      |
|----------------------------------------|-------------|-------|-------|-------|-------|-------|-------|-------|-------|-------|------|------|
|                                        | Fluid Type  |       |       |       |       |       |       |       |       |       |      |      |
|                                        | 70R1        | 70R1  | 70R3  | 70R3  | 70R3  | 70R1  | 70R1  | 70R1  | 70R1  | 70R1  | 70R1 | 70R1 |
| Parts                                  |             |       |       |       |       |       |       |       |       |       |      |      |
| TMPD/Ethylene glycol/                  |             |       |       |       |       |       |       |       |       |       |      |      |
| ethylene oxide.....                    | 33          | 24    | 33    | 25    | 38    | 26    | 26    | 33    | 25    | 19    |      |      |
| Diethylene glycol.....                 | 28          | 35    | 35    | 30    | 39    | 36    | 36    | 32    | 38    | 31    |      |      |
| 2-methylpentanol.....                  | 11          | 15    |       |       |       |       |       |       |       |       |      |      |
| Alcohol 750 <sup>1</sup> .....         | 12          | 15    |       |       |       |       |       | 18    | 20    |       |      |      |
| Ethylene glycol mono- butyl ether..... | 16          | 11    | 32    | 45    | 23    | 13    | 13    | 10    | 8     | 20    |      |      |
| Mixed amyl alcohols <sup>2</sup> ..... |             |       |       |       |       | 25    | 7     | 5     |       |       | 28   | 30   |
| Alcohol 3-58B <sup>3</sup> .....       |             |       |       |       |       |       |       |       |       |       |      |      |
| Finished fluid properties:             |             |       |       |       |       |       |       |       |       |       |      |      |
| -40° F. viscosity (centistokes).....   | 1,750       | 1,700 | 1,650 | 1,525 | 1,780 | 1,535 | 1,550 | 1,879 | 1,503 | 1,600 |      |      |
| Natural rubber swell (in.).....        | 0.031       | 0.056 | 0.025 | 0.061 | 0.031 | 0.030 | 0.031 | 0.040 | 0.039 | 0.057 |      |      |
| Percent evaporation.....               | 76          | 83    | 77    | 83    | 67    | 77    | 75    | 76    | 78    | 84    |      |      |

<sup>1</sup> C<sub>4</sub>-C<sub>8</sub> mixed primary and secondary alcohols.

<sup>2</sup> Approximately 64% n-amyl, 35% 2-Me-butyl, 1% n-butyl.

<sup>3</sup> 27% 2-methylpentanol, 10% isobutanol, 54% Alcohol 750.

various brake fluids generally varies from about 20% by weight to above 39% by weight. For the heavy duty type hydraulic brake fluids it is generally advantageous to utilize the trimethylpentanediol adduct in a concentration of from 21% by weight to about 31% by weight. For the extra heavy duty hydraulic brake fluids of the present invention it is generally advantageous to utilize a percentage range of about 25-30% by weight of the trimethylpentanediol adduct but higher concentrations can be utilized such as 28-39% by weight with the total composition still being capable of meeting the rigid SAE requirements. The brake fluids also contain a minor amount of antioxidant. While generally accepted antioxidants can be utilized in the brake fluid components of the instant invention it has been found that minor amounts, of up to 2%, of a 2-1 mixture of di-n-butylamine and 2,5-di-tert-butylhydroquinone together with tri-n-butylamine forms an especially useful antioxidant for the brake fluids of the instant invention.

The following examples illustrate various brake fluids of the instant invention but are not intended to be limitations thereof.

#### EXAMPLE 2

There was mixed 27 parts of the TMPD/ethylene glycol/ethylene oxide adduct as described above, 35 parts diethylene glycol, 8 parts by weight 2-methylpentanol, 15 parts by weight ethylene glycol monobutyl ether plus minor amounts of corrosion and oxidation inhibitors

75

(butyl amines and tert butyl hydroquinone) to produce a homogeneous, clear yellow fluid. This fluid was subjected to evaluation as a hydraulic fluid under SAE J70B specifications for 70R1 heavy duty brake fluids. This fluid met all requirements set forth by the specifications. The major results of this evaluation were as follows:

21-31% by weight the polyether adduct mixture; 21-31% Alcohol 3-58B, an alcohol mixture of about 27% 2-methylpentanol, 19% isobutanol, and 54% of various other C<sub>4</sub>-C<sub>8</sub> mixed primary and secondary alcohols (Alcohol 750);

(3)

21-31% by weight the polyether adduct mixture; 21-31% Alcohol 3-58B, an alcohol mixture of about 27% 2-methylpentanol, 19% isobutanol, and 54% of various other C<sub>4</sub>-C<sub>8</sub> mixed primary and secondary alcohols (Alcohol 750);

## 5

7-18% by weight ethylene glycol monobutyl ether;  
31-41% by weight diethylene glycol;  
0.1-1.0% by weight antioxidant.

(B) Extra heavy duty hydraulic brake fluid (70R3 type):

28-39% by weight the polyether adduct mixture;  
31-41% by weight diethylene glycol;  
20-40% by weight ethylene glycol monobutyl ether;  
0.1-1.0% by weight antioxidant.

The invention has been described in considerable detail with particular reference to certain preferred embodiments thereof, but it will be understood that variations and modifications can be effected within the spirit and scope of the invention as described hereinabove, and as defined in the appended claims.

We claim:

1. A hydraulic fluid consisting essentially of  
(A) about 25-35% by weight of a mixture of poly-  
ethers having the general formulae



and



wherein  $x$  is a whole number of from 1-10, the molar ratio of (1) to (2) being in the range of about 1/1 to 2/1,

(B) about 27-37% by weight diethylene glycol,  
(C) about 8-16% by weight 2-methylpentanol,  
(D) about 8-16% by weight mixed  $\text{C}_4\text{-C}_8$  primary and secondary alcohols,  
(E) about 8-16% by weight ethylene glycol mono- 35  
butyl ether, and  
(F) about 0.1-1.0% by weight antioxidant for inhibiting the oxidative degradation of the hydraulic fluid.

2. A hydraulic fluid consisting essentially of  
(A) about 28-39% by weight of a mixture of poly- 40  
ethers having the general formulae



and



wherein  $x$  is a whole number of from 1-10, the molar ratio of (1) to (2) being in the range of about 1/1 to 2/1,

(B) about 31-41% by weight diethylene glycol,  
(C) about 20-40% by weight ethylene glycol mono-  
butyl ether, and  
(D) about 0.1-1.0% by weight antioxidant for inhib- 50  
iting the oxidative degradation of the hydraulic fluid.

3. A hydraulic fluid consisting essentially of  
(A) about 21-31% by weight of a mixture of poly-  
ethers having the general formulae

## 6

(1)  $\text{HOCH}_2\text{CH}_2\text{O}(\text{CH}_2\text{CH}_2\text{O})_x\text{CH}_2\text{CH}_2\text{OH}$

and



wherein  $x$  is a whole number of from 1-10, the molar ratio of (1) to (2) being in the range of about 1/1 to 2/1,

(B) about 31-41% by weight diethylene glycol,  
(C) about 8-18% by weight ethylene glycol mono-  
butyl ether,  
(D) about 5-25% by weight of  $\text{C}_4\text{-C}_8$  primary and  
secondary alcohols,  
(E) about 5-25% by weight of mixed amyl alcohols,  
and

(F) about 0.1-1.0% by weight antioxidant for inhib-  
iting the oxidative degradation of the hydraulic fluid.

4. A hydraulic fluid consisting essentially of  
(A) about 21-31% by weight of a mixture of poly-  
ethers having the general formulae



and



wherein  $x$  is a whole number of from 1-10, the molar ratio of (1) to (2) being in the range of about 1/1 to 2/1,

(B) about 21-31% by weight of an alcohol mixture  
consisting essentially of

(1) about 27 wt. percent 2-methylpentanol  
(2) about 19 wt. percent isobutanol, and  
(3) about 54 wt. percent of  $\text{C}_4\text{-C}_8$  primary and  
secondary alcohols,

(C) about 31-41% by weight diethylene glycol,  
(D) about 7-18% by weight ethylene glycol mono-  
butyl ether, and  
(E) about 0.1-1.0% by weight antioxidant for inhib-  
iting the oxidative degradation of the hydraulic fluid.

## References Cited

## UNITED STATES PATENTS

|           |         |                            |
|-----------|---------|----------------------------|
| 2,425,755 | 8/1947  | Roberts et al.             |
| 3,062,747 | 11/1962 | Fife et al. ----- 252-73   |
| 3,324,035 | 6/1967  | Nankee et al. ----- 252-73 |
| 3,341,456 | 9/1967  | Sawyer ----- 252-75        |
| 3,346,501 | 10/1967 | Boehmer ----- 252-73       |

55 LEON D. ROSDOL, Primary Examiner

D. SILVERSTEIN, Assistant Examiner

U.S. Cl. X.R.